

Oct. 25, 1927.

1,646,468

K. WARGA

DECORATED GLASS OBJECTS AND METHOD OF PROTECTING  
THE DECORATED SURFACES  
Filed April 2, 1924

*Fig. 1.*



*Fig. 2.*



INVENTOR.

Kalman Warga  
BY  
Redding, Greeley, O'Dea & Campbell  
ATTORNEYS.

Patented Oct. 25, 1927.

1,646,468

# UNITED STATES PATENT OFFICE.

KALMAN WARGA, OF NEW YORK, N. Y., ASSIGNOR TO PYROCOLOR CORPORATION, OF NEW YORK, N.Y., A CORPORATION OF VIRGINIA.

## DECORATED GLASS OBJECTS AND METHOD OF PROTECTING THE DECORATED SURFACES.

Application filed April 2, 1924. Serial No. 703,827.

The decorated surfaces of glass objects are subjected to atmospheric, acid and mechanical erosion, especially when mounted in exposed situations, which quickly destroy 5 the appearance and function of the decoration whether it be letters, symbols or fanciful designs. So serious are the effects named, that it has become the best practice to lead in colored decorative sections. This solution 10 is expensive and lacks some of the advantages to be derived from the use of an integral glass object having the decorations applied to its surface. The principal object of the present invention is to provide 15 a method of decorating glass surfaces in distinctive color and then applying a protective coating to such surface which is atmospheric and acid-proof and protects the color from injury through physical causes. Still 20 another object is to provide a simple and inexpensive method of decorating the surface of clear glass sheets with color which is fixed thereon and then applying a protective coating over the color which makes the 25 glass object translucent without changing the true hue of the color when viewed with a light background, and yet insuring the most vivid display possible for a light source of given candlepower. Still another object 30 of the invention is to provide a process for decorating a glass surface and protecting the decoration at the time the glass is heated to a temperature necessary for working into desired form, such as spherical or curved. 35 In practicing the invention one or more colors may be employed in decorating a glass surface and the colors may be applied in accordance with the process set forth in Letters Patent of the United States No. 40 1,283,606 dated November 5, 1918, or merely stencilled on the surface. Next it is proposed, in accordance with the invention, to apply over the colors and, usually, over the entire surrounding surface of the glass a 45 white enamel which has a lower fusing point than the glass. This enamel is of such properties as to render crystal glass translucent and protect the color against atmospheric, acid and physical attacks. More 50 specifically, the preferred method consists in applying one or more colors to a glass surface, in accordance with the process described in said Patent No. 1,283,606, treating the surface with a protective enamel and then shaping the glass, all of these steps be-

ing performed successively but under a single heating of the glass. To render such process feasible the fusing point of the color is fixed lower than that of the enamel and the fusing point of the enamel is fixed lower 60 than that of the glass so that the color is first fired without disturbing the enamel and the glass is worked without danger.

The invention will be described in greater detail in connection with the drawing which 65 shows, merely by way of illustration, a crystal glass globe whose rear surface has been treated in accordance with the process and in which:

Figure 1 is a view in elevation of the 70 globe.

Figure 2 is a fragmentary sectional view through the lettering thereon and taken on the plane indicated by the line 2—2 of Figure 1 and looking in the direction of the 75 arrows.

While the invention is not to be limited, in its broader aspect, to the use of crystal glass nor to the manner in which the decoration is applied to the surface, the preferred 80 embodiment contemplates the use of ordinary clear glass and the firing of color thereon. In carrying out the process a flat sheet of clear glass *a* may have applied to its surface suitable colored lettering, symbols or fanciful decorations by either stenciling or by the method described in Letters Patent of the United States No. 1,283,- 85 606. In this method the design for the color is printed upon the gummed face of the 90 decalcomania paper and is dusted with the desired color. Powdered flux is mixed with the color in such proportions as to fix the fusing temperature at the desired point. The decalcomania paper bearing the color 95 design is then applied to the surface of the glass sheet *a* which has been treated with a size and the paper removed leaving the design transferred, as indicated at *b*. Any gum from the decalcomania paper may be 100 washed off with water from the design transferred to the glass whose surface is allowed to dry.

A white enamel backing *c* is then spread over the design *b* and the surrounding surface of the glass *a*. This white enamel is so prepared as to fix its fusing point at less than that of the glass but somewhat higher than that of the firing point for the color, although the fusing point of the enamel is 110

such that it is within the working range of the glass.

Following the treatment described the glass is then heated to the firing point of 5 the color so that it is fixed on the glass in the manner pointed out in said Patent No. 1,283,606. A continuance of heat brings the glass to a temperature where it may be worked into any desired cross sectional form.

10 In the illustrated embodiment it is proposed to shape it into an integral sphere to serve as a globe for use over an electric lamp. After having given the glass plate the desired form the temperature is gradually re-

15 duced to atmospheric.

The resulting object is one in which the crystal glass is rendered translucent by the enamel backing *c* but this backing is of such nature as to insure the most vivid light effect 20 for a given candle-power. The color of the decoration *b* is protected by the coating from atmospheric, acid and physical disintegration and has been found in practice to give its true hue when viewed with a light source 25 back of it. The process is economical, saving the repeated heating and treating of the glass in different stages rather than in completing all of the operations described at a single heating.

30 As pointed out before, the design might be applied by stenciling on the rear surface of

the glass and the enamel coating then applied and the same degree of protection secured.

What I claim is:

1. The method of decorating glass objects 35 and protecting the decoration which consists in printing the color design on the surface by decalcomania transfer, applying a coating of weather and acid-proof enamel over the color and then heating the glass to a temperature sufficient to fire the color, the material of the color and of the enamel having been previously so compounded as to fuse at a temperature below the fusing point 40 of the glass.

2. The method of decorating glass objects and protecting the decoration which consists in printing the color design on the surface by decalcomania transfer, applying a coating of weather and acid-proof enamel 50 over the color and then heating the glass to a temperature sufficient to fire the color, the material of the color and of the enamel having been previously so compounded as to fuse at a temperature below the fusing point 55 of the glass, and then shaping the glass during such heating to the desired cross-sectional form.

This specification signed this 28th day of March A. D. 1924.

KALMAN WARGA.